

## UNITED STATES PATENT OFFICE

2,029,969

SILK YARN PREPARED FROM NATURAL  
SILK IN THE GUM

Leo Wallerstein, Rowland A. Gale, and Thomas G. Hawley, Jr., New York, N. Y., assignors to Wallerstein Company Inc., a corporation of New York

No Drawing. Application April 26, 1934,  
Serial No. 722,505

## 1 Claim. (Cl. 117—53)

The present invention relates to the preparation of yarns and threads from natural silk in gum. Raw silk as exported to this country from Japan and from other silk producing centers consists of fine strands of the silk protein, fibroin, each of which is encased in a coating of the silk gum termed sericin. This gum detracts from the appearance of the silk fibres, but is left on such fibres throughout the textile forming operations to give such fibres body and permit them to be more readily handled.

In textile forming processes, the skeins are usually subjected to a winding process, which consists of the removal of the filaments from the skein onto suitable carriers, then the individual filaments are combined together with a little twist in a process which is termed the 5B operation and then one or more of these doubled filaments may be highly twisted from 30 up to 85 or 10 more turns per inch to give a suitable yarn or fibre for knitting or weaving purposes.

Although the sericin or gum coating on the filaments advantageously lends body to the fibroin, it is disadvantageous in that it gives a wiry characteristic to the filaments, which wiry characteristic offers a substantial resistance to twisting. This resistance increases as the amount of twist and the number of threads twisted together is increased. This wiry quality of the individual 30 silk filaments tends to cause kinking and prevents a uniform packing together of the filaments when twisted or thrown which uniform packing is most desirable in the production of high grade yarns.

When the twisted yarns are to be utilized for knitting purposes, they are wound on frusto-conical shapes known to the trade simply as cones, this process being ordinarily known as coning. Due to the wiry quality of the threads, however, 40 it is difficult to place these threads uniformly upon cones and the thread upon being taken off the cone will not run smoothly therefrom, but will rather tend to slip and jump off, giving rise to tangles. This necessitates frequent adjustments of the machine together with attended stopping and loss of time by the operator. And, moreover, a considerable loss of silk in the form of waste occurs.

On the other hand, in the weaving industry, where the yarn for the filler or weft is placed upon suitable quills or bobbins, carried in the shuttles, it is most important to maintain a desirable tension of the filler as it is placed in the sheds formed by the warp. Due to the wiry characteristics of the natural silk yarn carrying its gum, it is diffi-

cult to maintain this tension since the silk tends to readily slip and jump off the quills and bobbins with the same disadvantageous effects as occur in the knitting process, above described.

Some attempts have been made to alleviate this wiry property of the natural silk in gum by impregnating such silk with various combinations of soap and oils. In general, the more wiry the silk to be treated, the more soap and oil required, and it was generally found difficult to place sufficient soap and oil in the silk to decrease or alleviate the wiry property in a most satisfactory manner.

In addition, an object of the present invention is to provide a yarn which will most satisfactorily lend itself to winding, doubling, and twisting operations, which will be largely devoid of the objectionable wiry qualities of natural silk in gum, and which at the same time will not necessarily carry objectionable quantities of soap and oil.

Another object is to provide improved knitting and weaving processes, in which assurance is had that the silk yarn or filaments may be uniformly and properly taken off the cones, spindles, and/or quills during the textile-forming operation, without tendency toward tangles, uneven tension and other undesirable effects.

Other objects will appear during the course of the following specification.

In accomplishing the above objects, it has been found that the wiry property of the natural silk in gum may be largely alleviated by impregnating the silk before the textile operations with a proteolytic enzyme preparation, at such temperatures, and pH values that no substantial amount of the gum is removable.

It has been found most desirable to utilize soaking baths at temperatures below 50° C. and at pH values ranging from 4 to 10. The period of impregnation may vary from 15 to 30 minutes up to overnight or 18 hours depending on the enzyme concentration. After the impregnation, the silk fibres are preferably dehydrated mechanically as much as possible, as by centrifuging and then are air-dried.

After drying, the fibres are subjected to the textile-forming operations, above described.

Silk treated in this manner may be wound, doubled, and twisted to form highly twisted multi-filament yarns, of most high quality. The individual strands of these yarns will lay closely packed together in a most uniform fashion and the tendency toward kinkiness and unevenness will be greatly decreased.

In addition the treated yarn will lay most satis-

factorily upon cones, quills, and/or bobbins, to give a uniform tension and to run off smoothly and evenly without slippage or tangling during the operation of the textile machines.

5 The enzyme preparation is generally utilized in conjunction with soap and/or oils to insure proper penetration and lubrication.

Various protease preparations may be used in carrying out the process, such as protease preparations derived from micro-organisms which under suitable culture conditions develop proteolytic enzymes, as for instance, preparations derived from *Aspergillus oryzae*, from cultivation of bacteria, such as *B. mesentericus*, *B. mycoides*, 10 or *B. subtilis*, or *Mucor delemar*, *Amylomyces*, *Rouxii*, *Penecillium*, and so forth. Other suitable proteolytic enzymes may be used, such as papain, bromelin, malt enzymes, trypsin, pancreatin or pepsin. Suitable mixtures of the 15 above described enzymes may also be used.

As examples in carrying out the process, one may proceed as follows:

Example 1.—100 pounds of raw silk are soaked from 30 minutes to 1 hour in a bath or 25 solution consisting of 400 pounds of water in which have been dissolved 50 pounds of the bacterial enzyme preparation, 1 pound of sodium sulfite for effecting a suitable pH, and 1 pound of sulfonated oil, this latter material being used 30 to effect a better penetration, or as it is technically called, a wetting-out of the bire, though it will be understood that other penetrants can be used for effecting this wetting-out such as a small amount of soap.

35 If the soaking period is increased, the amount of enzyme may be decreased, as for example, with overnight soaking only half as much enzyme is required.

Other suitable pH regulators, for instance, 40 sodium carbonate or bicarbonate, or a mixture thereof, may be used instead of the sodium sulfite referred to.

Emulsions of common soaking oils, such as 45 neat's foot oil, may also be used in conjunction with enzymes.

The temperature at which this process is carried out may be advantageously varied with the time consumed in the operation, the nature or origin of the silk, the nature of the particular

enzyme employed, and the presence of other constituents, such as pH regulators. However, we generally employ this process at room temperature, that is, from 60 to 85° F.

The silk is then removed from the enzyme bath 5 and the adhering liquor is removed in any suitable manner, as by centrifuging, and after the centrifuging step, the silk fibres are dried at a low temperature by an air blast or any other suitable method.

Example 2.—100 pounds of 13/15 Japan white silk in the gum are soaked for 30 minutes at room temperature in 400 pounds of water solution containing 5 pounds of papain, 4 pounds of sulfonated oil, 0.05 pound of potassium cyanide, and 15 2 pounds of mono-sodium phosphate. It is then centrifuged and air dried.

Example 3.—100 pounds of 13/15 Japan white silk in the gum are soaked for 30 minutes at room temperature in 400 pounds of water solution containing 5 pounds of pancreatin, and 1 pound of sodium sulfite with suitable penetrants and oils. It is then centrifuged and air dried.

The yarns as prepared above may be most satisfactorily wound, doubled, twisted, knitted, 25 and/or woven without the many disadvantages due to the wiry characteristics of the natural silk which soaking solely with oils and/or soap does not satisfactorily alleviate.

The present application is a continuation in 30 part of copending application Serial No. 606,286, filed April 19, 1932, and is similar in subject matter to copending applications Serial No. 722,504 and Nos. 722,506 to 722,508 all inclusive, filed April 26, 1934.

The present application is particularly directed to highly twisted yarns of decreased kinkiness or tendency to snarl.

What is claimed is:

Highly twisted silk yarns for weaving and knitting, comprising natural silk in gum, said yarn being rendered more flexible and with lessened tendency toward kinkiness and unevenness by impregnation with a proteolytic enzyme preparation without removal of the gum, the yarn 45 being dry and containing said preparation.

LEO WALLERSTEIN.

ROWLAND A. GALE.

THOMAS G. HAWLEY, JR.